

## UNITED STATES PATENT OFFICE

LUDWIG J. CHRISTMANN, OF JERSEY CITY, AND STUART A. FALCONER, OF ELIZABETH,  
NEW JERSEY, ASSIGNEES TO AMERICAN CYANAMID COMPANY, OF NEW YORK, N. Y.,  
A CORPORATION OF MAINE

## FLOTATION RECOVERY OF MINERALS

No Drawing.

Application filed January 9, 1930. Serial No. 419,733.

The object of this invention is the successful separation of oxide minerals from ores containing the same. Many reagents are known which are promoters for sulfide ores but not all sulfide reagents are effective in the flotation of so-called oxidized minerals. On the other hand, reagents for oxidized minerals will in general assist in the flotation of sulfides.

10 By an oxidized mineral we mean a heavy metal such as lead, zinc, copper, etc., in combination with elements or groups of elements other than sulfur.

We have discovered that the alkaline metal 15 salts of hydroaromatic xanthates, for example, potassium cyclohexyl xanthate, potassium methyl cyclohexyl xanthate, are effective reagents in the flotation of oxide ores. We prefer to use these reagents in combination 20 with other reagents. These other reagents may be varied considerably, but a hydroaromatic xanthate is always essential in the practice of our invention.

The structural formula for this type of reagent is:



30 where Me is a metal of the alkaline type, such as sodium, potassium, ammonium, calcium, etc. R is an alkyl group, such as methyl, 35 ethyl, etc., or an aryl group, such as phenyl, naphthyl, etc., or hydrogen. R may be placed in the ortho, meta or para positions.

We have prepared cyclohexyl xanthate by the following method:

40 50 g. of cyclohexylanol (hexalin) and 15 g. of potassium hydroxide were heated under reflux until the KOH was in solution. The solution was stirred, cooled and 200 cc. of ethyl ether added. The mixture was placed in an ice bath and 15 cc. of carbon bisulfide in 100 cc. of ether were slowly added. The precipitate of potassium cyclohexyl xanthate was filtered, washed with ether, and allowed to air-dry. To purify the above it was dissolved in acetone, the undissolved portion

filtered off, and the filtrate diluted with benzol and the precipitate thrown down was a cream colored product of high purity.

The potassium o. methylcyclohexyl xanthate was prepared in an analogous manner.

The following examples are illustrative of the practice of our invention on the oxidized lead ore of the North Lily Mine of the International Smelting Company.

1200 g. of ore, 1200 cc. of water and 5.0 lbs. 60 of crude monoammonium phosphate per ton of ore were ground in a laboratory rod mill for 12 minutes. The mesh of the feed is 60% minus 200. The rod mill charge was transferred to a laboratory mineral separation sub- 65 area machine and diluted to 22% solids. The reagents were added to the machine and a mineralized froth collected for 20 minutes.

## Reagents in pounds per ton to mill

70  
Ammo. phos. (crude mono-ammonium phosphate) 5.0 5.0

## To flotation machine

75  
Ammonium n. dibutyl dithiophosphate 1.25 1.25  
Potassium cyclohexyl xanthate 4.0  
Percent lead in heads 26.6 26.6  
Percent lead in concentrates 38.2 36.6 80  
Percent lead in tails 19.59 2.11  
Percent lead in recovered 54.5 97.7

Under the same conditions a run made with potassium o. methylcyclohexyl xanthate showed:

## Reagents in pounds per ton to mill

85  
Ammo. phos. (crude mono-ammonium phosphate) 5.0 5.0

## To flotation machine

90  
Ammonium n. dibutyl dithiophosphate 1.25 1.25  
Potassium o. methylcyclohexyl xanthate 4.0 95  
Percent lead in heads 26.6 26.3  
Percent lead in concentrates 38.2 47.45  
Percent lead in tails 19.59 5.38  
Percent lead in recovered 54.5 89.8 100

In the practice of our invention we may vary the details considerably from the illustrations given above. We may use other reagents besides the ammonium n. dibutyl 5 dithiophosphate and the crude monoammonium phosphate. For example, we may use other xanthates in place of dibutyl dithiophosphate or other dithiophosphates. The essential feature of our invention is the use 10 of a hydroaromatic xanthate of which potassium cyclohexyl xanthate and potassium o. methylcyclohexyl xanthates are types. Other homologues of cyclohexyl xanthate may be used. We consider that this type of 15 hydroaromatic xanthate nucleus is responsible for the increased activity of these xanthates over the ordinary xanthates of the aliphatic series which are now in use.

What we claim is:

- 20 1. A method of recovering minerals from ores which comprises subjecting an oxidized ore to a froth flotation operation in the presence of a salt of a cyclohexyl xanthate as a promotor.
- 25 2. A method of recovering minerals from ores which comprises subjecting an oxidized ore to a froth flotation operation in the presence of a salt of a substituted xanthate as a promotor.
- 30 3. A method of recovering minerals from ores which comprises subjecting an oxidized ore to a froth flotation operation in the presence of potassium methyl cyclohexyl xanthate as a promotor.
- 35 4. A method of recovering minerals from ores which comprises subjecting an oxidized ore to a froth flotation operation in the presence of a promotor having the following structural formula:



50 where Me is a metal and R is an aryl or alkyl group or hydrogen and R may be in ortho, meta or para position.

- 55 5. A method of recovering minerals from ores which comprises subjecting an oxidized ore to a froth flotation operation in the presence of a salt of a cyclohexyl xanthate as a promotor in conjunction with another promotor.

- 60 6. A method of recovering minerals from ores which comprises subjecting an oxidized ore to a froth flotation operation in the presence of a salt of a cyclohexyl xanthate as a promotor in conjunction with a dithiophosphate.

- 65 7. A method of recovering minerals from ores which comprises subjecting an oxidized ore to a froth flotation operation in the pres-

ence of a salt of a cyclohexyl xanthate as a promotor in conjunction with another promotor, and a conditioner.

In testimony whereof, we have hereunto subscribed our names this 2nd day of January, 1930.

LUDWIG J. CHRISTMANN.  
S. A. FALCONER.

75

80

85

90

95

100

105

110

115

120

125

130